# EUROPEAN PATENT SPECIFICATION

(11) **EP 2 878 914 B1**
(45) Date of publication and mention of the grant of the patent: **20.02.2019**
(21) Application number: 14460076.4
(22) Date of filing: 23.10.2014
(51) Int. Cl.: F41H 1/02, F41H 5/04

(54) **Anti-trauma pad**
Unterlage für Traumaschutz
Couche anti-trauma

(30) Priority: 01.12.2013 PL 40633113
(43) Date of publication of application: 03.06.2015
(73) Proprietor: Instytut Technologii Bezpieczeñstwa "Moratex", 90-965 Lódz (PL)
(72) Inventor: Zielinska, Dorota, 94-058 Lodz (PL); Olszewska, Karolina, 91367-Lodz (PL); Struszczyk, Marcin H., 95-070 Ruda Bugaj (PL); Delczyk-Olejniczak, Bogumila, 91-149 Lodz (PL); Wierzbicki, Lukasz, 06-400 Ciechanow (PL); Kozlowska, Joanna, 04-534 Warszawa (PL); Leonowicz, Marcin, 03-977 Warszawa (PL)

(56) References cited:
- WO-A1-01/81853
- WO-A1-90/14942
- CN-A- 102 692 161
- US-A- 5 604 022

## Description

The subject of the invention is the elastomeric anti-trauma pad dedicated for use in the personal armours, together with a ballistic panel.

Ballistic panels that save lives or limit the wearer's injuries after a hit of a projectile from firearms are widely known and used, A ballistic panel undergoes deflection upon a projectile hit, causing deformation of a basis, which transfers into the severity of an injury.

Since ballistic panels are heavy and expensive, providing adequate security and usage comfort without increasing the load is an important issue.

A ballistic pad forming a starting point for the present invention is known from WO 01/81853 A1.

To improve the usage comfort, sometimes the additional elastomer inserts of foam structure are applied together with the ballistic panel.

The above object is achieved by the features of appended independent claim 1.

The essence of the solution according to the invention consists in developing a light structure strongly absorbing the energy, to be used as a pad under a ballistic panel, causing a decrease in the deflection of ballistic panel upon a shot.

The anti-trauma pad is a flexible plate made of an elastomeric material, comprising a closed inner chamber which occupies up to 90% vol. of the plate, wherein one exterior side of the plate is flat, while the other is equipped with the arrangement of protrusions, distributed evenly over its entire area.

Number of the protrusions amounts from 1500 up to 3000 / m², and the minimum thickness of the pad measured between the protrusions is not less than 7mm, while including the protrusions it is up to 27 mm maximum. Preferably, the height of the protrusions is from 2 up to 15 mm.

The pad may contain a dilation liquid of up to 90% vol., introduced uniformly into the structure of the elastomer and/or to the inner chamber.

As an example of the dilation liquid, a suspension is used, which contains from 15 up to 30% vol. of fumed silica of the grain diameter of 5 to 15 nm with 70 up to 85% vol. of the polypropylene glycol.

Preferably, the elastomeric material of pad comprises an additive in the form of spheres in an amount of up to 5%, filled with an inert gas, while the diameter of the spheres fits in the range from 1 nm up to 990 µm.

Reduction in deflection of a ballistic panel for use in personal armours has a significant impact on reducing the internal injuries upon a shot.

The deformation of base upon a hit with the 7,62x39 mm PS bullet, determined according to the requirements of PN-V-87001:2011 Standard is reduced by 60-70% for the arrangement of ballistic composite with the pad, compared to a test performed on the panel without the pad.

The anti-trauma pad according to the invention is shown in the drawings, where **Fig.1** shows a view of the pad from the bottom, and **Fig.2** - a fragment of the pad's cross-section.

The pad has one outer side flat **1**, while the other side has protrusions **2** which are identical, regularly spaced and positioned next to each other. Inside the plate there is a closed chamber **3** of a shape corresponding to the outer outline of the plate and filled with the dilation liquid.

### Embodiment example I.

The pad in the form of plate with one side flat, and the other with protrusions in the shape of truncated pyramids, manufactured of equal amounts of two components of silicone ZA 22 MOULD (resin base and accelerator) from Amod, Poland, has an internal chamber containing the dilatation liquid of the following composition: 25% vol. of fumed silica of 7 nm diameter and 75% vol. of the polypropylene glycol. The anti-trauma pad with dimensions of 300x250 mm, maximum thickness 17 mm and minimum thickness 8,6 mm, has 168 protrusions. The pad contains 300g of dilatation liquid and the total mass of pad is 980 g.

Deformation of basis of the system of pad with a panel of ballistic composite made of non-woven sheets of UHMWPE fibres, shot with 7,62x39 mm PS bullets, according to the PN-V-87000:2011 Standard, at the temperature of 23°C, exhibits the maximum deflection of 9,3 mm, while the reference ballistic panel without the pad - 30,8 mm.

Reduction of deflection compared to the reference model is 69%.

### Embodiment example II.

The pad as that in example I, containing the 1,2% addition of microspheres 461 DET 40 d25 from AKZO Nobel, Holland in the structure of silicon, with the total maximum thickness of 16 mm and minimum of 8 mm, has total mass of 800 g, including 280 g of dilatation liquid.

The panel together with the pad, exhibit maximum deflection of 12,0 mm, when shot with 7,62x39 mm PS bullet.

Reduction in deflection, compared to the reference ballistic panel without the pad is 61%.

## Claims

1. An anti-trauma pad made of elastomeric material, dedicated for use in personal armours together with ballistic panels, ***characterised in that*** the anti-trauma pad is formed of elastomeric material comprising a closed inner chamber (**3**), wherein the top exterior surface of the pad (**1**) is flat, while the bottom one comprises a system of protrusions (**2**) distributed evenly over its entire area in the amount of from 1500 to 3000 /m² and of a height from 2 mm to 15 mm.

2. The pad according to claim 1, ***characterised in that*** its minimum thickness between protrusions (**2**) is not less than 7 mm, and the maximum including the protrusions (**2**) is up to 27 mm.

3. The pad according to claim 1, ***characterised in that*** the protrusions (**2**) on its bottom side have the form of truncated pyramids.

4. The pad according to claim 1, ***characterised in that**,* silicon is used as the elastomeric material.

5. The pad according to claim 1, ***characterised in that*** the elastomeric material in its structure comprises spheres in the amount of up to 5% of weight, filled with the inert gas.

6. The pad according to claim 5, ***characterised in that*** the diameters of the spheres are in the range of 1 nm to 990 µm.

7. The pad according to claim 1, ***characterised in that*** the closed inner chamber (**3**) occupies up to 90 % of the plate volume.

8. The pad according to claim 1, ***characterised in that*** it comprises up to 90% vol. of dilation fluid.

9. The pad according to claim 8, ***characterised in that*** the dilation fluid comprises a suspension of 15-30% vol. of fumed silica, of grain diameter in the range of 5-15 nm with 70-85% vol. of polypropylene glycol.

10. The pad according to claim 8, ***characterised in that*** the dilation fluid is homogenously introduced into the structure of elastomer and/or to the internal closed chamber (**3**).

## Patentansprüche

1. Unterlage für Traumaschutz aus Elastomerwerkstoff zur Anwendung in persönlicher Schutzausrüstung inklusive ballistischer Platten, ***dadurch gekennzeichnet,* dass** sie die Form einer Elastomerplatte beinhaltend eine geschlossene Innenplatte (**3**) hat, wobei die obere Außenoberfläche der Platte (**1**) flach ist und die untere ein System von gleichmäßig auf der ganzen Oberfläche verteilten Vorsprünge (**2**) in einer Menge von 1.500 bis 3.000 /m² und mit einer Höhe von 2 mm bis 15 mm.

2. Unterlage nach Anspruch 1, ***dadurch gekennzeichnet,* dass** ihre minimale Dicke zwischen den Vorsprüngen (**2**) mindestens 7 mm, und ihre maximale Dicke samt den Vorsprüngen (**2**) bis zu 27 mm beträgt.

3. Unterlage nach Anspruch 1, ***dadurch gekennzeichnet,* dass** die Vorsprünge (**2**) auf ihrer Unterseite die Form eines Pyramidenstumpfes haben.

4. Unterlage nach Anspruch 1, ***dadurch gekennzeichnet,* dass** als Elastomerwerkstoff Silikon verwendet wird.

5. Unterlage nach Anspruch 1, ***dadurch gekennzeichnet,* dass** der Elastomerwerkstoff in seiner Struktur mit Inertgas befüllten Sphären in einer Menge von bis zu 5 Gew.-% enthält.

6. Unterlage nach Anspruch 5, ***dadurch gekennzeichnet,* dass** die Durchmesser der Sphären im Bereich von nm bis 990 µm liegen.

7. Unterlage nach Anspruch 1, ***dadurch gekennzeichnet,* dass** die geschlossene Innenkammer (**3**) 90 Vol.-% der Platte darstellt.

8. Unterlage nach Anspruch 1, ***dadurch gekennzeichnet,* dass** sie bis zu 90% Dilatationsflüssigkeit enthält.

9. Unterlage nach Anspruch 1,8 ***dadurch gekennzeichnet,* dass** die Dilatationsflüssigkeit eine Suspension aus pyrogenem Siliziumoxid mit einem Korndurchmesser von 5-15 nm in einer Menge von 15-30 Vol.-% und Polypropylenglykol in einer Menge von 70-85 Vol.-% ist.

10. Unterlage nach Anspruch 1,8 ***dadurch gekennzeichnet,* dass** die Dilatationsflüssigkeit homogen in die Struktur des Elastomers und/oder in die geschlossene Innenkammer (**3**) eingeführt wurde.

## Revendications

1. Couche anti-trauma est faite du matériau élastomère, destinée pour l'utilisation dans les protections individuelles y compris les plaques balistiques, ***caractérisée en ce qu'***elle a la forme de plaque élastomère comprenant une chambre intérieure fermée (**3**), et la surface supérieure extérieure de la plaque (**1**) est plate et la surface inférieure comprend un système de saillies réparties uniformément sur toute la surface (**2**) dont le nombre est de 1500 à 3000 /m² et la hauteur de 2 mm à 15 mm.

2. Couche selon la revendication 1, ***caractérisée en ce que*** son épaisseur minimalne parmi les saillies (**2**) n'est pas moindre de 7 mm, et au maximum avec les saillies (**2**) jusqu'à 27 mm.

3. Couche selon la revendication 1, ***caractérisée en ce que*** les saillies (**2**) sur sa partie inférieure ont la forme de pyramides coupées.

4. Couche selon la revendication 1, ***caractérisée en ce que*** le silicone est utilisé en tant que matériau élastomère.

5. Couche selon la revendication 1, ***caractérisée en ce que*** le matériau élastomère contient dans sa structure des sphères jusqu'à 5% en poids remplies d'un gaz inerte.

6. Couche selon la revendication 5, ***caractérisée en ce que*** les diamètres de sphères sont compris dans les limites de 1 nm à 990 µm.

7. Couche selon la revendication 1, ***caractérisée en ce que*** la chambre intérieure fermée (**3**) constitue jusqu'à 90 % en volume de la plaque.

8. Couche selon la revendication 1, ***caractérisée en ce qu'***elle contient jusqu'à 90% du liquide de dilatation.

9. Couche selon les revendications 1,8 ***caractérisée en ce que*** le le liquide de dilatation est une suspension 15-30% en vol. de silice de pyrogénation avec le diamiètre de grain entre 5-15 nm et 70-85% en vol. de propylène glycol.

10. Couche selon les revendications 1,8 ***caractérisée en ce que*** le liquide de dilatation est introduit uniformément dans la structure d'élastomère et/ou dans la chambre intérieure fermée. (**3**).
